

April 28, 1936.

H. D. GEYER

2,038,727

GRINDING WHEEL

Filed June 20, 1935

2 Sheets-Sheet 1



Fig. 1

Fig. 2



INVENTOR  
Harvey D. Geyer  
BY  
Spencer Hardman & Fehr  
HIS ATTORNEYS

April 28, 1936.

H. D. GEYER

2,038,727

GRINDING WHEEL

Filed June 20, 1935

2 Sheets-Sheet 2



Fig. 4



Fig. 5



Fig. 6

INVENTOR  
Harvey D. Geyer  
BY  
Spencer Hardman & Fehr  
HIS ATTORNEYS

## UNITED STATES PATENT OFFICE

2,038,727

## GRINDING WHEEL

Harvey D. Geyer, Dayton, Ohio, assignor to General Motors Corporation, Detroit, Mich., a corporation of Delaware

Application June 20, 1935, Serial No. 27,477

5 Claims. (Cl. 51—278)

This invention relates to rigid abrasive bodies, such as grinding wheels of carborundum, emery, or other well known abrasive materials, and means for securely fixing such abrasive bodies upon a supporting metal back plate or other metal support for the non-metallic abrasive material.

An object of this invention is to provide an improved means and method for rigidly fixing such abrasive bodies to a supporting metal back plate, such as steel, which will give greater surety against the abrasive body, such as a grinding wheel, breaking apart and flying off when rotated at very high speeds in use. This provides greater safety for the operator.

Another object of the invention is to provide means for mounting disk grinding wheels upon the metal back plate which fixes the wheel to its rotating shaft, which means will permit the use of the wheel when it is worn to a smaller thickness than is permissible with such disk grinding wheels mounted by means now in general use.

Further objects and advantages of the present invention will be apparent from the following description, reference being had to the accompanying drawings wherein a preferred embodiment of the present invention is clearly shown.

In the drawings:

Fig. 1 is a face view of a finished disk grinding wheel bonded to its supporting back plate according to this invention.

Fig. 2 is a section taken on line 2—2 of Fig. 1.

Fig. 3 illustrates a step in the method of this invention, and shows the spray-coating of the back surface of the abrasive wheel.

Fig. 4 shows the coated abrasive wheel and the coated metal back plate with their coated surfaces in juxtaposition, illustrating how these two coated surfaces are applied one to the other prior to the bonding step of the method.

Figs. 5 and 6 illustrate in a diagrammatic manner an apparatus which may be used for carrying out the bonding step of the method.

Fig. 5 is a plan view of a turn-table which holds the abrasive wheel and its back plate in assembled position during the heating step and during the pressing and cooling step of the method.

Fig. 6 is a vertical section taken on line 6—6 of Fig. 5 and shows both the position of the wheel assembly during the heating step and during the pressing and cooling step.

Similar reference characters refer to similar parts throughout the several figures of the drawings.

55 10 designates the rigid non-metallic abrasive

wheel itself, which may be of carborundum, emery, or any other similar and well known abrasive material.

11 is the supporting metal back plate to which the abrasive wheel 10 is strongly surface bonded by means of the intervening metal layer 12 which adheres very strongly both to the contacting surface of wheel 10 and the plate 11. Plate 11 is preferably of steel and is shown as having an integral hub 13 by which the wheel assembly may be 10 suitably fixed to its rotating shaft. Of course plate 11 may be a flat plate bolted or otherwise suitably fixed to a separate hub member. This invention relates only to the means and method of securely fixing the abrasive body 10 to the adjacent surface of plate 11.

In following the method of this invention, the back surface of the abrasive wheel 10 is first spray coated with molten metal which may be lead, tin, zinc, copper, or other suitable metal or a suitable alloy of such metals, to form the relatively thin strongly adhering metal coating 15 shown in Fig. 4. A coating 16 of a similar suitable metal is also applied to the surface of plate 11 which is to be bonded to the wheel 10. The abrasive wheel 10 and the metal plate 11, having been thus coated with the relatively thin coats 15 and 16 respectively, are then assembled together in the proper relative positions and heated to a temperature sufficient to soften or fuse the two metal coats 15 and 16 and pressure is applied to force the two coated surfaces 15 and 16 together while they are in an alloyable or fusible condition, and they are then cooled while this pressure is being maintained. This results in the two contacting coats 30 35 15 and 16 being firmly bonded together in a manner similar to soldering. When this is done the non-metallic abrasive wheel 10 is strongly bonded to the metal back plate 11 and the wheel is ready for use.

40 Fig. 3 shows one apparatus and method of spray-coating the abrasive wheel 10 with the spray coat 15. The supply of liquid coating metal 20 for forming the spray coat 15 is maintained in molten condition in container 21 by 45 a suitable gas burner 22. Directly above container 21 is mounted a rotating shaft 23 having a series of thin metal spraying disks 24 fixed thereto, these disks being of a metal, such as steel, having a melting point sufficiently high to 50 prevent damage thereto by insertion in the molten metal 20. The level of the molten metal 20 is kept at such a point that the lower portions of disks 24 are immersed therein. Now when shaft 23 is power driven at a suitably high speed 55

the disks 24 will pick up the molten metal and throw it off radially in fine particles thus giving something which may be called a metal mist 25. The wheel 10 is rotatably mounted upon the 5 journal 26 directly in the path of the metal spray 25, hence when wheel 10 is slowly rotated about journal 26 by any suitable means (not shown) the under surface thereof will be coated with a uniformly applied spray coat 15. The 10 fine metal particles are thrown by centrifugal force with high speed against the normally rough surface of the abrasive body 10 while they are yet plastic and hence these metal particles penetrate into the smallest crevices and minute cavities 15 in the abrasive material and upon immediately solidifying therein are firmly locked or keyed to the abrasive material. By thus substantially keying the first layer of individual small particles of metal to the abrasive surface 20 and subsequently keying these first applied particles of metal to each other by the particles thrown later against them to form the coating 15, it has been found that such coating 15 will adhere very strongly to the abrasive material 25 and cannot be stripped therefrom without shearing the metal itself. It is desirable to spray the metal particles from disks 24 through an atmosphere of non-oxidizing or reducing gas in order to prevent partial oxidation of the particles during 30 transit or after they have been deposited upon the abrasive material. For this purpose the housing is preferably kept filled with a suitable non-oxidizing or reducing atmosphere during the spraying operation. The chamber 27 is maintained heated to a suitable temperature by 35 any suitable heating means, such as by the electric heating coils 28. As soon as the sprayed metal particles pass out of chamber 27 through the opening 29 they cool rapidly and hence substantially immediately solidify upon striking the relatively cool abrasive wheel 10.

The metal coating 16 is separately applied to the metal back plate 11 by any simple and well known method, such as by dipping the suitably 45 cleaned and fluxed plate 11 into molten metal and immediately removing same. Preferably a number of grinding wheels 10 and backing plates 11 are coated with coats 15 and 16 respectively, and these parts are subsequently assembled to 50 together to form the units shown in Fig. 2 by the bonding operation illustrated in Figs. 5 and 6.

Fig. 5 shows a turn-table 40 for supporting and handling a series of grinding wheels 10 when set loosely upon their back plates 11 during the 55 heating step and also during the compressing step of the bonding operation. Turn-table 40 has a series of radial arms 41 each having an end fork 42 thereon adapted to receive the hub portion 12 when the back plates 11 are set upon the ends of arms 41 with the wheels 10 thereupon as shown in Fig. 5. While the loosely assembled units 10 and 11 are in the two positions "A" and "B" of Fig. 5, the desired amount of heat is applied by the small gas burners 43 to 60 bring the metal coatings 15 and 16 up to the desired bonding temperature. The loosely assembled unit is then shifted to position "C" where it is located between the press plunger 45 and press table 46. At this point press plunger 70 45 is caused to descend upon the top surface of wheel 10 and thus press the contacting metal-coated surfaces of wheel 10 and plate 11 together while the metal coatings 15 and 16 thereon are in a soft or semi-plastic state. These 75 coatings are strongly bonded or alloyed together

upon cooling while the pressure of plunger 45 is being maintained. The press plunger 45 is then raised and the now assembled wheel unit shifted to position D of Fig. 5, where it is removed as the finished unit shown in Fig. 2.

While the apparatus shown in Figs. 5 and 6 heats the metal coatings 15 and 16 to the desired point prior to the main pressure being applied to bond these coatings together, if desired the heating step and pressing step of this invention 10 may be carried on simultaneously. However it is preferred in any case to maintain the application of the pressure until the bonding coating has solidified by cooling.

While this method has been illustrated and 15 described in connection with bonding a disk grinding wheel to its supporting back plate, it is readily adaptable for use in bonding other kinds of grinding wheels or non-metallic abrasive bodies to shafts or metal adapters of any desired 20 design, or for bonding any other ceramic or similar body such as tile to a supporting metal sheet or plate.

While the embodiment of the present invention as herein disclosed, constitutes a preferred 25 form, it is to be understood that other forms might be adopted, all coming within the scope of the claims which follow.

What is claimed is as follows:

1. A grinding wheel of non-metallic abrasive 30 material having a metal support therefor surface bonded thereto over substantially the entire radial surface on one side of said wheel by means of an intervening metal layer which adheres strongly to both the abrasive material and said 35 metal support.

2. The steps in the method of rigidly fixing a rigid non-metallic abrasive body to a metal back, comprising: providing a strongly adhering spray coat of relatively low-melting metal upon said 40 abrasive body by throwing fine particles of molten metal with high speed against said body and thereby causing strong adherence of said spray coat, providing a relatively low-melting metal coat upon said metal back, then pressing the 45 abrasive body against the metal back in such manner as to bring their coated surfaces into intimate pressure contact at a temperature sufficient to partially fuse and bond said contacting metal coats together, then cooling the assembly 50 while maintaining said pressure contact.

3. The steps in the method of rigidly fixing a rigid non-metallic abrasive body to a metal back, comprising: providing a strongly adhering, relatively thin metal coat upon said abrasive body, 55 providing a relatively thin metal coat upon said metal back, said metal coats both having a lower-melting point than the metal of said back and having a bonding affinity for each other, then pressing the abrasive body against the metal back 60 in such manner as to bring their coated surfaces into intimate pressure contact at a temperature sufficient to bond said contacting metal coats together, then cooling the assembly while maintaining said pressure contact.

4. The steps in the method of rigidly fixing an abrasive grinding wheel upon a metal back plate, comprising: spraying molten metal upon one surface of said wheel to give it a relatively thin strongly adhering metal coat, separately providing a relatively thin metal coat upon said metal back plate, both of said metal coats having a lower melting point than the metal of said back plate, then pressing the coated surface of the grinding wheel against the coated surface of the back 75

plate at such a temperature as will fuse or alloy said two contacting metal coats together and provide a strong metal bond between said grinding wheel and back plate.

5. The steps in the method of rigidly fixing a ceramic body to a metal back, comprising: providing a strongly adhering relatively thin metal

coat upon said ceramic body, providing a relatively thin metal coat upon said metal back, then pressing the two metal-coated surfaces of said ceramic body and metal back together at a temperature sufficiently high to strongly bond said contacting metal coats together. <sup>5</sup>

HARVEY D. GEYER.